

G. C. WESTBY.  
 PROCESS AND APPARATUS FOR SULFATIZING METALLIFEROUS ORES.  
 APPLICATION FILED APR. 10, 1917.

1,266,732.

Patented May 21, 1918.

*Fig. 1.*



*Fig. 2.*



*Fig. 3.*



*Fig. 4.*

George C. Westby  
 By Chas. E. Riordan  
 Attorney

# UNITED STATES PATENT OFFICE.

GEORGE C. WESTBY, OF LUDWIG, NEVADA, ASSIGNOR TO WESTERN PROCESS COMPANY,  
A CORPORATION OF MAINE.

## PROCESS AND APPARATUS FOR SULFATIZING METALLIFEROUS ORES.

1,266,732.

Specification of Letters Patent. Patented May 21, 1918.

Application filed April 10, 1917. Serial No. 160,934.

*To all whom it may concern:*

Be it known that I, GEORGE C. WESTBY, a citizen of the United States, residing at Ludwig, in the county of Lyon and State of Nevada, have invented certain new and useful Improvements in Processes and Apparatus for Sulfatizing Metalliferous Ores, of which the following is a full, clear, and exact specification.

10 This invention relates to a process for sulfatizing metalliferous ores and simultaneously extracting the metal values therefrom by leaching wherein the ores are subjected simultaneously to the action of sulfurous gases and an aqueous liquid.

20 In accordance with my invention the ores are subjected while wet with an aqueous liquid to the action of a sulfatizing reagent or reagents comprising principally sulfurous gases and oxidizing gases. In practice I cause a current of liquid to pass through the ore, preferably in a downward direction, while causing a current of the gaseous reagents to pass through the ore in the opposite direction. In treating "fines", however, by ordinary means, I have found that it is practically impossible to carry out the invention by ordinary means, the interstices between the particles of ore rapidly becoming filled and the mass of wetted ore becoming so dense as to render the passage of gas therethrough exceedingly difficult. My present invention consists in a process and apparatus which I have devised more especially for the treatment of finely comminuted metalliferous ores with liquid and gas simultaneously to effect their sulfatization and the lixiviation of the metal values therefrom.

40 My process and apparatus are illustrated by the accompanying drawings, in which;

Figure 1 shows in broken section and side elevation a view of an apparatus in accordance therewith;

45 Fig. 2 shows in plan and partial section, a view of a detail of Fig. 1;

Fig. 3 shows in plan a modified form of the detail shown in Fig. 2, and;

50 Fig. 4 shows a cross-section through the element shown by Fig. 3.

In accordance with my present invention, instead of forming the ore fines into a relatively large and dense mass for its treatment with liquid and gas, I cause it to form in a large number of heaps or masses of low

height and resting upon supports which will allow the passage of gas. I also provide for the agitation and discharge of these small heaps, the material contained in them falling upon similar supports arranged below those from which it is discharged, on which lower supports it is again subjected to the action of the reagent.

As illustrated in the accompanying drawing my device comprises an inclosed reaction chamber 10 provided with suitable charging hoppers 11, at its top and with an inclined bottom 12 and a discharge opening 13 at its base, the discharge opening being closed by a suitable movable cut-off 14. 65 Near the bottom of said chamber an inlet conduit 15 having an upturned end 16 within the chamber, above which is arranged a hood or distributor 17 provides for the admission of sulfurous gases, for example, 70 those proceeding from a smelter furnace. Within this conduit I also provide a steam inlet nozzle 18, through which I may force steam, which causes the device to act as an injector and accelerates the movement of 75 the gas. At the top of the reaction chamber I provide an outlet pipe 19 for the gas, which may discharge into the atmosphere or be forced through other reagent chambers, 80 as desired.

At the top of the reaction chamber I also provide for the introduction of water or other liquid, which enters through the inlet pipe 20 and is distributed by suitable sprays 21.

Within the reaction chamber, for the support of the ores treated, I provide between the water distributors at the top and the gas inlet at the bottom a series of transverse supports 22. As shown in Figs. 1 and 2 of 95 the drawing these transverse supports each consists of two spaced members or slats 23, 23 between which extends a rope 24, ordinarily not tightly tensed. This rope is anchored at one end to one wall of the reaction chamber 10 by means of a suitable plate 25, and at its other end passes through an opening in the opposite wall of the chamber and is attached to the soft iron core 26 of a suitable solenoid 27. These solenoids are 100 connected in suitable electrical circuits 28, 28.

Near the bottom of the reaction chamber I provide a discharge opening 29 for the liquid which collects therein, which may pass to a suitable tank for the separation of the 110

metal values or may be forced by means of pump 30 and pipe 31 to a second reaction chamber. In carrying out my invention I charge the metalliferous ore fines treated, 5 such as, for example, oxidized cupriferous ores, or other cupriferous, zinkiferous and manganiferous ores capable of sulfatization into the hoppers 11, from which they are discharged into the chambers from the supports 22. These supports are arranged in 10 series in staggered relation or quincuncially, so that the material in falling descends from one to another and forms in low heaps upon the height of these heaps being determined 15 by the angle of rest of the specific material.

After charging the supports in the reaction chamber with the material I pass thereinto a current of sulfurous gases, preferably containing a relatively high proportion of 20 oxidizing agent, such as oxygen, air, oxidizing nitrous gas or the like. I simultaneously inject steam through the steam inlet 18, this accelerating the movement of the sulfurous gases and simultaneously introducing aqueous vapor into the reaction chamber. I also cause a regulated flow of aqueous liquid 25 through the pipe 20 and distributer 21 over at the top of the reaction chamber, which descends through the numerous small heaps of ore simultaneously with the ascent of the gas and water vapor. The water vapor, in rising, condenses and the condensate is added to the aqueous liquid and together with it passes downward through the small masses 30 of ore wetting them and leaching soluble metal values therefrom. By reason of the interspaces between the side members of the supports and the central agitating member the gases and liquid pass not only over the 35 surfaces of the small heaps of air, but also pass therethrough.

After the passage of the gaseous and liquid reagents for some time I close the electric circuit through the solenoids, thereby suddenly tensing the central ropes which form the vibrating members of the transverse supports. This sudden tensing of the rope causes the material on the supports to be 45 violently shaken and to fall upon those below, thereby preventing the ore from becoming too densely compacted and exposing fresh surfaces to the action of the reagent.

The treated ore from the lower transverse supports falls into the contracted bottom of 50 the reaction chamber, from which it may be discharged through opening 13.

The simultaneous action of the sulfurous gases, which contain oxidizing reagents, the steam and the water effects a sulfatization of 55 the ore and the leaching of the soluble metal values therefrom. The liquid which collects in the bottom of the reaction chamber contains these soluble metal values, and may be withdrawn through pipe 29 to be discharged 60 to a suitable precipitation system or to be

used in the treatment of the same or of a fresh batch of ore. The aqueous liquid supplied through the pipe 20 and distributer 21 may also be the liquid derived from previous treatment of ore.

In Figs. 3 and 4 I have illustrated a modified form of transverse support in which the vibrator rope of the form shown in Fig. 2 is replaced by a rotatable member journaled in the walls of the reaction chamber. In 70 these figures 10' indicates opposite walls of the reaction chamber, between which extend the spaced fixed members 33, 33. Between these members and spaced therefrom to permit of the passage of gas and of its own rotation is the rotatable longitudinal member 34, the cylindrical ends 35, 35 of which are journaled in the walls 10', 10'. The rotation or oscillation of this central member of each 75 cross support is effected by means of any 80 suitable mechanical device, such as, for example, the sprocket wall 36.

In operation I may, if desired, effect the operation of the vibrating members of the transverse supports in successive sets or 85 zones. Thus if the supports be grouped into three zones I may first effect the operation of the agitating members of the lowermost zone, which will cause the greater part of the material supported by them to fall into the 90 bottom of the reaction chamber. I may then operate the agitating members of the next higher zone, which will cause the material on the supports in this zone to fall on the supports in the lowermost zone. Operation 95 of the vibrating members of the supports in the uppermost zone then causes the material thereon to descend to the second zone, and finally the supports in the uppermost zone are charged from the charging 100 hoppers. The arrangement of the vibrating 105 devices necessary for such operation is illustrated by Fig. 1 of the drawings, wherein groups of the solenoids operating the vibrating members and forming zones are shown 110 in independently controlled circuits.

Having thus described my invention what I claim as new and desire to secure by Letters Patent is:—

1. In a process for sulfatizing metalliferous fines, arranging said fines in series of low heaps in relatively staggered relation within an inclosed chamber, passing a gaseous sulfatizing reagent and steam upwardly through said heaps and over their 115 surfaces and simultaneously wetting and leaching the fines in said heaps with an aqueous liquid, and vibrating said heaps, thereby exposing fresh surfaces to the action of the reagents.

2. An apparatus for sulfatizing ore fines comprising an inclosed tower, a series of transverse supports within said tower in relatively staggered arrangement, said supports permitting passage of gas and being 120 125 130

provided with agitating means, means for introducing gas and water vapor near the base of said tower and a gas outlet at its top, means for introducing water near the top of the tower, and means for charging and discharging ore therefrom.

5 3. In a tower for treating ore fines simultaneously with liquid and a sulfatizing gas, a plurality of spaced transverse supports, 10 each comprising a pair of fixed, spaced, parallel members and a vibrating member between and spaced from them, and means for operating said vibrating members.

4. In a process of sulfatizing metalliferous fines, arranging said fines in a series of 15 low heaps in relatively staggered relation within a closed tower, passing a gaseous sulfatizing reagent together with steam through and around said heaps and successively through the closed ore chambers, 20 simultaneously wetting and leaching the fines and said heaps by means of condensed steam and the condensing spray of an aqueous liquor.

25 5. In a process for sulfatizing metalliferous fines consisting in arranging said fines in a series of low heaps in relatively staggered relation within an inclosed tower, passing a gaseous sulfatizing reagent together with steam through and around said heaps

and successively through the closed ore chambers, vibrating said heaps and simultaneously wetting and leaching said fines during said vibration by means of the aqueous liquor formed.

35

6. In a process for sulfatizing metalliferous fines consisting in charging said fines at the top of a closed tower to a set of staggered shelves arranged to form the ore fines into low heaps and cause the material to gradually advance and slowly drop consecutively from point to point to the discharge while sulfurous gases and steam are forced into the apparatus together with sufficient aqueous spray to condense the steam thus sulfatizing and leaching the soluble values from the ore.

7. In a tower for treating ore fines simultaneously with liquid and a sulfatizing gas, a plurality of spaced transverse supports, 50 each comprising a pair of fixed, spaced, parallel members, a rope capable of being tensed between said members, and means for tensing said rope.

8. An apparatus as specified in claim 2, 55 wherein the transverse supports are divided into parallel operative zones and their agitating members operated in said zones successively from the bottom upwardly.

GEORGE C. WESTBY.